

1

3,012,967

## MINERAL OIL COMPOSITION

Samuel J. Leonardi, Pitman, and Edward A. Oberright,  
Woodbury, N.J., assignors to Socony Mobil Oil Company, Inc., a corporation of New York  
No Drawing. Filed July 26, 1957, Ser. No. 674,279  
4 Claims. (Cl. 252—48.2)

This invention has to do with the stabilization of petroleum fractions, particularly of lubricating oils. More specifically, it relates to petroleum fractions having incorporated therein certain combinations of additives in order to greatly inhibit the oxidative deterioration of such fractions.

It is well known that petroleum oil fractions refined for use as lubricants are subject to oxidative deterioration under conditions of use in modern combustion engines. The oxidation products which are formed in the oil are acidic in nature and exert a corrosive effect on the metal parts with which the oil comes in contact. Alloy bearings, such as copper-lead, silver-cadmium, nickel-cadmium, etc., which are widely used, are particularly subject to attack by the acidic oxidation products formed in the oil in use. Furthermore, these oxidation products produce formations of varnish and sludge on the engine surfaces which lower the operating efficiency of the engine. Also, due to oxidation effects, the viscosity of the oil is changed in use so that proper lubrication of the engine parts is not obtained. In the case of turbine oils, the problem of oxidation is increased since the oil normally becomes contaminated with water.

It is an object of this invention, therefore, to provide a class of addition agents for petroleum oil fractions which are capable of substantially inhibiting the oxidative deterioration of such fractions. A further object is to provide petroleum compositions, such as lubricating oils, which are highly stabilized against oxidation under the conditions of use.

It is an object of this invention to stabilize mineral lubricating oils against the deleterious effects of oxidation.

It is a related object to provide lubricating oil compositions containing certain advantageous combinations of additives, hereinafter described.

Other and further objects will become apparent from the following description of the invention.

It has been found that the foregoing objects can be realized by incorporating into a lubricating oil fraction, a small amount of each of: (1) an aromatic hydroperoxide having a hydroperoxy group attached to an alpha carbon atom of an aryl nucleus thereof, and (2) an acid whose dissociation constant in water is at least about  $1.0 \times 10^{-5}$ .

It is to be understood that no claim is made herein to an oil containing a hydroperoxide (1) in the absence of an acid (2), since such are shown by Watkins in U.S. Patent No. 2,470,276. Similarly, no claim is made to an oil containing an acid (2) in the absence of a hydroperoxide (1), for such are shown by Bulkley et al. in U.S. Patent No. 2,248,848. In neither of these patents, nor in any other prior art known to us, is there a showing of an oil containing a hydroperoxide (1) and an acid (2). The latter oils are greatly superior to oils containing only one of the said two additives.

The aromatic hydroperoxides (1) of this invention are represented by the following general formulae:

(a)



2

and

(b)



wherein A is an aryl group, such as benzene, naphthalene and biphenyl, or is an alkaryl group wherein the alkyl (or cycloalkyl) substituent can be such as methyl, ethyl, butyl or cyclohexyl; R<sub>1</sub> and R<sub>2</sub> are any combination of hydrogen, cycloalkyl, alkyl, aryl, alkaryl, cycloalkylaryl or aralkyl; and R<sub>3</sub> is an alkyl group of 2 or 3 carbon atoms whose terminal carbon is connected to the aryl group A.

Representative of the hydroperoxides contemplated herein and designated by general Formula a, are:  $\alpha$ -cumyl hydroperoxide;  $\alpha$ -p-xylyl hydroperoxide; p-cymene hydroperoxide;  $\alpha,\alpha$ -dimethylbenzyl hydroperoxide;  $\alpha,\alpha$ -dimethyl-p-methylbenzyl hydroperoxide; and  $\alpha,\alpha$ -dimethyl-p-isopropylbenzyl hydroperoxide.

Representative of the hydroperoxides contemplated herein and designated by general Formula b, are: tetralin hydroperoxide and hydrindene hydroperoxide.

Of these compounds, the  $\alpha$ -cumyl,  $\alpha$ -p-xylyl, and tetralin hydroperoxides are preferred herein.

As indicated above, the second additive used in the new compositions is an acid whose dissociation constant in water is at least  $1.0 \times 10^{-5}$ . It is to be understood that the first dissociation constant of a polybasic acid (K<sub>a1</sub>) will have such a value. Typical of such acids are: acetic, ma-

leic, oxalic, propionic, phosphoric, phosphorous, pyrophosphoric, picric, sulfuric, sulfurous, benzoic, pyromellitic, mellitic, benzene sulfonic, p-toluene sulfonic, and hydroxydecanoic. Preferred of such acids are phosphoric acid and p-toluene sulfonic acid.

Typical examples of hydroperoxides contemplated herein are revealed by the following:

### EXAMPLE I

Commercial alpha-cumyl hydroperoxide was purified as follows: The sodium salt of alpha-cumyl hydroperoxide was precipitated when the hydroperoxide was contacted with aqueous sodium hydroxide at temperatures below 77° F. The resulting reaction mixture was contacted with benzene and the sodium salt was filtered off with suction. The sodium salt was washed with benzene, dried, and suspended with water. The hydroperoxide was liberated by adding carbon dioxide to the sodium salt, and was extracted with petroleum ether. The ether was then removed by distillation under vacuum. The residue contained 9.87 percent active oxygen (by iodometric titration) and its refractive index ( $n_D^{20}$ ) was 1.5253. Theoretical values for alpha-cumyl hydroperoxide are 10.52 percent active oxygen and 1.5242 ( $n_D^{20}$ ), respectively.

### EXAMPLE II

Alpha p-xylyl hydroperoxide was prepared by the following procedure:

Para-xylene was oxidized by bubbling oxygen therethrough at temperatures between 60 and 65° C., until a peroxide number determination indicated that one percent of the p-xylene charge had been converted to the hydroperoxide. The reaction mixture was then contacted with aqueous sodium hydroxide, whereupon the sodium salt of the hydroperoxide precipitated. The salt was recovered by filtration. The salt was suspended in ether and the resulting mixture was acidified with dilute aqueous hydrochloric acid cooled to 0° C., in order to obtain the hydroperoxide dissolved in the ether layer.

The ether layer was washed with sodium carbonate to remove traces of acid, dried with magnesium sulfate and

the ether was removed by evaporation. By twice purifying the p-xylene reaction product through the sodium salt, the hydroperoxide was concentrated to about 55 percent purity. Peroxide number determinations indicated .4 percent of active oxygen in the purified product; the theoretical value for active oxygen is 11.6 percent.

Oxidation stabilities of blends of a mineral oil containing combinations of the hydroperoxides and acids contemplated herein, were determined. This was in contrast to corresponding tests on the oil alone, the oil containing a hydroperoxide but not containing an acid, and the oil containing an acid but not containing a hydroperoxide. The test used is an oxidation stability test mentioned after that described by Larsen, Thorpe and Armfield in Industrial and Engineering Chemistry 34, 89-93 (1942). In this test oxygen is dispersed by means of a sintered glass bubbler through the oil at 300°. The degree of deterioration of the oil is determined by measuring the amount of oxygen that reacts with the oil. The results are reported in hours required for absorption of two liters of oxygen per 100 grams of oil. The longer the time for this absorption to take place, the more stable the oil.

The oil used in the tests was a highly acid-refined oil having the following properties:

|                                |        |
|--------------------------------|--------|
| Viscosity, at 100° F. (S.U.S.) | 135.2  |
| Viscosity, at 210° F. (S.U.S.) | 42.5   |
| Viscosity index                | 108    |
| pour point, ° F.               | +30    |
| specific gravity, $d_4^{20}$   | 0.8588 |
| refractive index, $n_D^{20}$   | 1.4722 |

Results of the oxidation stability tests are given in Table I following:

Table I

| Additive                    | Cone., per cent by Weight | Hours Required for Absorption of 2 Liters O <sub>2</sub> /100 gms. Oil Blend |
|-----------------------------|---------------------------|------------------------------------------------------------------------------|
| None                        |                           | 1.2                                                                          |
| Phosphoric Acid             | 0.12                      | 1.1                                                                          |
| p-Toluene Sulfonic Acid     | 0.03                      | 1.2                                                                          |
| Alpha-Cumyl Hydroperoxide   | 7.5                       | 1.6                                                                          |
| Alpha-Cumyl Hydroperoxide   | 7.5                       | 70                                                                           |
| Phosphoric Acid             | 0.12                      |                                                                              |
| Alpha-Cumyl Hydroperoxide   | 7.5                       | 92                                                                           |
| p-Toluene Sulfonic Acid     | 0.03                      |                                                                              |
| Alpha-p-Xylyl Hydroperoxide | 10                        | 294                                                                          |
| p-Toluene Sulfonic Acid     | 0.06                      |                                                                              |

\* 10 percent of product of Example II containing 55 percent of hydroperoxide.

Data given in Table I reveal that the combination of an acid and a hydroperoxide is surprisingly superior to the results obtained with only one of the said additives.

The amounts of acid and hydroperoxide to be added to a petroleum oil fraction will vary somewhat with the particular oil fraction and the conditions of use. In general, the amount of acid will be from 0.001 to about 3.0 percent by weight of the oil, preferably 0.01 to 1.0 percent. Correspondingly, the amount of hydroperoxide will generally vary from about 0.1 to about 10 percent by weight of the oil; 1.0 to 8 percent is the preferred range. The additives of this invention may, of course, be added to petroleum fractions along with other additive agents designed to improve various other characteristics of such fractions, for example, pour point depressants, extreme pressure agents, detergents and the like.

Although the invention has been illustrated herein by the use of specific examples of my additive products and in a particular petroleum medium, it is not intended that the scope of this invention be in any way limited thereby, but only as shown in the accompanying claims.

We claim:

1. A petroleum lubricating oil subject to oxidative deterioration and containing (1) a minor amount, from about 1.0 to 8 percent by weight of the oil, of a hydroperoxide selected from the group consisting of  $\alpha$ -cumyl hydroperoxide and  $\alpha$ , $\alpha$ -xylyl hydroperoxide and tetralin hydroperoxide, and (2) a minor amount, from about 0.01 to 1.0 percent by weight of the oil, of an acid selected from the group consisting of phosphoric acid and p-toluene sulfonic acid.

2. A petroleum lubricating oil subject to oxidative deterioration and containing about 7.5 percent by weight of alpha-cumyl hydroperoxide and about 0.12 percent by weight of phosphoric acid.

3. A petroleum lubricating oil subject to oxidative deterioration and containing about 7.5 percent by weight of alpha-cumyl hydroperoxide and about 0.03 percent by weight of p-toluene sulfonic acid.

4. A petroleum lubricating oil subject to oxidative deterioration and containing about 6 percent by weight of alpha-p-xylyl hydroperoxide and about 0.06 percent by weight of p-toluene sulfonic acid.

References Cited in the file of this patent

UNITED STATES PATENTS

|           |               |               |
|-----------|---------------|---------------|
| 2,119,240 | Lyons         | May 31, 1938  |
| 2,248,848 | Bulkley       | July 8, 1941  |
| 2,249,340 | Wilson et al. | July 15, 1941 |
| 2,470,276 | Watkins       | May 17, 1949  |
| 2,773,906 | Emerson       | Dec. 11, 1956 |